

## UNITED STATES PATENT OFFICE

1,920,953

## STAIN RESISTING WROUGHT ARTICLE

Frederick M. Becket, New York, N. Y., assignor to  
 Electro Metallurgical Company, a Corporation  
 of West Virginia

No Drawing. Application March 14, 1930  
 Serial No. 435,957

6 Claims. (Cl. 148—12)

The invention relates to articles fabricated from stain-resisting alloys having the very high degree of workability necessary to adapt them to deep-drawing operations.

For purposes which require a stain-resisting metal of fairly high strength and moderate cost, the usual materials at the present time are alloys consisting principally of iron, but containing enough chromium to impart the desired stability of surface. As is well known, these alloys (the carbon percentage being sufficiently low) possess to a remarkable degree the ability to withstand various corrosive influences. It has been found that the capacity of such alloys for deep-drawing can be markedly improved by an addition of nickel, and low-carbon alloys containing approximately 18% of chromium and 8% to 14% of nickel, with most of the balance iron, are the best deep-drawing alloys of this class now in commercial use.

The alloys with which the present invention is concerned are adapted to the same class of uses as the iron-chromium-nickel alloys referred to above. Whereas the iron-chromium-nickel alloys usually contain only fractional percentages of manganese, the alloys of the present invention contain several percent of this element. On the other hand the alloys with which this application is concerned do not comprise nickel as an essential component, though additions of nickel are by no means precluded.

For the purposes of the present invention, the alloys should contain at least about 16% of chromium, and at least about 5% of manganese. The upper limit of the chromium range contemplated herein is about 22%. As a rule I prefer to place the chromium percentage between 17% and 21%. With the chromium in the vicinity of 20%, at least about 6% of manganese is desirable. The manganese improves the shock resistance, Erichsen value and deep-drawing properties. The maximum effect in this direction appears to be attained when the manganese content reaches 15% or so, but higher percentages of manganese, up to at least 20%, have no detrimental effect, and are quite unobjectionable unless on economic grounds. Taking all factors into account, a manganese content of 8% to 12% is preferred for most purposes.

In the softest and most ductile grades of the alloys under discussion, carbon is not an essential constituent, and it is present only because it is commercially impossible completely to exclude it. Alloys with less than 0.12% carbon are especially suitable for some uses, and this figure may

be set as a practical maximum for the grades of alloy which are most nearly carbon-free. Greater strength and hardness can be imparted by the incorporation of more carbon, and without much impairment of the stain-resistance and workability, but for the applications of the alloy herein contemplated, the carbon is preferably held below a maximum of about 0.3%.

Deoxidizing and refining agents may of course be added to the metal, as in standard metallurgical practice, and doubtless there are other elements which may be present in greater or smaller proportion without destroying the useful properties of the metal, or may even improve it for certain purposes.

In the following table certain of the properties of specific alloys in the wrought condition are shown:

| Analysis |       |      | Heat treatment                               | Izod impact foot pounds | Erichsen value | 75 |
|----------|-------|------|----------------------------------------------|-------------------------|----------------|----|
| Cr       | Mn    | C    |                                              |                         |                | 70 |
| 17.88    | 8.26  | 0.07 | Heated 5 min. at 1050° C. and water quenched | 112.0                   | 10.35          | 80 |
|          |       |      | Heated 5 min. at 1050° C. and air cooled     | 77.0                    | 10.30          |    |
| 17.55    | 10.48 | 0.07 | Heated 5 min. at 1150° C. and water quenched | 112.0                   | 10.10          |    |
|          |       |      | Heated 5 min. at 1150° C. and air cooled     | 85.0                    | 9.40           | 85 |
| 18.99    | 12.41 | 0.08 | Heated 5 min. at 1150° C. and water quenched | 119.5                   | 8.80           |    |
|          |       |      | Heated 5 min. at 1150° C. and air cooled     | 72.0                    | 8.60           |    |
| 17.54    | 14.77 | 0.09 | Heated 5 min. at 1150° C. and water quenched | 120.0                   | 10.00          |    |
|          |       |      | Heated 5 min. at 1150° C. and air cooled     | 115.5                   | 9.20           | 90 |
| 18.34    | 11.75 | 0.18 | Heated 5 min. at 1150° C. and water quenched | 120.0                   | 10.6           |    |
|          |       |      | Heated 5 min. at 1150° C. and air cooled     | 35.5                    | 10.2           |    |

Each of the alloys was subjected, in both the quenched and the air-cooled conditions, to other physical tests as indicated below. The ranges of the numbers obtained were as follows:

Yield point----- 48,000 to 62,000 lbs. 100 per. sq. in.  
 Maximum stress----- 89,800 to 126,000 lbs. per. sq. in.  
 Elongation in 2 inches----- 25% to 48%  
 Reduction of area----- 25.1% to 70.0% 105

The Brinell numbers fall between 149 and 166 except in the case of the last alloy in the table, containing 0.18% carbon. It registered 187 as quenched and 196 as air-cooled. Each alloy was also subjected to the Erichsen test without pre- 110

vious heat-treatment, i. e. as rolled. The lowest value recorded was 8.75.

When immersed in cold dilute nitric acid (20 cc. 68%  $\text{HNO}_3$  + 80 cc. water), polished samples of 5 the various alloys did not in any case lose as much as 0.0001 grams per square centimeter per hour.

Polished samples of the tabulated alloys were 10 in no case affected by the standard salt spray test in 7 days; and when subjected to the Brearley test with copper sulphate solution, no sample precipitated a visible deposit of copper.

It has already been indicated in the prior art 15 that certain iron-chromium manganese alloys are forgeable, and that certain alloys composed of these elements are stain-resistant and ductile 20 after heating and quenching. It will of course be understood that a metal may be truly said to be ductile even though it is practically devoid of deep-drawing properties. Deep-drawing requires 25 a high degree of ductility, combined with toughness and strength, and in the investigation of a new alloy the possession of deep-drawing quality can only be shown by actual trial, regardless of the behavior of the metal in any usual physical 30 test. A fortiori, forging being the simplest form of metal working and deep-drawing one of the most difficult forms, forgeability is by no means invariably accompanied by deep-drawing properties. 35 So far as I am aware, there is no published statement that any stain-resisting iron-chromium-manganese alloy possesses deep-drawing properties, nor is there any published statement that any such alloy can be rendered ductile without quenching. The alloys of the present invention, in the air-cooled condition, have deep-drawing properties comparable with those of the most workable stain-resisting iron-chromium-nickel alloys when the latter have been heat-treated in the manner which influences their 40 workability most favorably.

An important advantage of the iron-chromium-manganese alloys described herein, from a commercial point of view, is that very little difficulty is encountered in casting them into 45 clean ingots. With the stain-resisting iron-chromium-nickel alloys, clean metal is only consistently obtained by those thoroughly familiar with their peculiarities, and only by the most careful work. As will be readily understood, inclusions 50 in the metal are highly detrimental to its stain resistance.

I claim:—

1. A stain-resistant article having properties 55 imparted by deep-drawing and by cooling from a temperature between about 1050° C. and about

1150° C.; said article being composed of an alloy obtaining iron, chromium, manganese, and carbon; and said alloy having substantially the composition: 16% to 22% chromium, 6% to 14% manganese, not more than about 0.3% carbon, 80 remainder iron.

2. An article having properties imparted by air-cooling from a temperature between about 1050° C. and about 1150° C.; said properties including an Erichsen number greater than about 85 8.5, and stain-resistance; said article being composed of an alloy containing iron, chromium, manganese, and carbon; and said alloy having substantially the composition: 16% to 22% chromium, 6% to 14% manganese, not more than about 0.3% carbon, remainder iron. 90

3. Method of producing stain-resisting, shock-resisting, ductile articles, which comprises deep-drawing an alloy containing iron, chromium, manganese, and carbon in substantially the proportions: 16% to 22% chromium, 6% to 14% manganese, not more than about 0.3% carbon, remainder iron and small amounts of incidental impurities; heating the deformed alloy to a temperature between about 1050° C. and about 1150° 100 C.; and thereafter cooling the alloy.

4. Method of producing stain-resisting, shock-resisting articles having an Erichsen number greater than about 8.5, which comprises deep-drawing an iron-chromium-manganese-carbon 105 alloy having substantially the composition: 16% to 22% chromium, 6% to 14% manganese, not more than about 0.3% carbon, remainder iron; heating said alloy to a temperature between about 1050° C. and about 1150° C.; and thereafter 110 quenching the alloy.

5. An article having properties imparted by deep-drawing and by rapid cooling from a temperature between about 1050° C. and about 1150° C., said properties including an Erichsen number 115 greater than about 8.5, and stain-resistance; said article being composed of an alloy containing iron, chromium, manganese, and carbon; and said alloy having substantially the composition: 16% to 22% chromium, 6% to 14% manganese, not more than about 0.3% carbon, remainder iron.

6. A stain-resistant deep-drawn article composed of an alloy steel having substantially the composition: 17% to 21% chromium, 6% to 14% manganese, carbon, the carbon content being not 125 more than about 0.12%, the balance iron; which steel has been rapidly cooled from a temperature between about 1050° C. and 1150° C.

FREDERICK M. BECKET. 130